# EUROPEAN PATENT SPECIFICATION

(11) **EP 1 752 523 B1**
(45) Date of publication and mention of the grant of the patent: **31.12.2008**
(21) Application number: 05023239.6
(22) Date of filing: 25.10.2005
(51) Int. Cl.: C11C 5/00, C11C 5/02

(54) **Candle body composition for colored flame candles and use thereof**
Kerzenkörperzusammensetzung mit gefärbter Flamme und Verwendung dieser Zusammensetzung
Composition pour corps de bougie à flamme de couleur et son utilisation

(30) Priority: 08.08.2005 CN 200510087783
(43) Date of publication of application: 14.02.2007
(73) Proprietor: Jiande Jiaxuan Articles Co., Ltd., Jiande City Zhejiang 311600 (CN)
(72) Inventor: LI, Hua, Jiande City Zhejiang Province 311600 (CN); Lu, Xin, Jiande City Zhejiang Province 311600 (CN)
(74) Representative: Neumann, Ditmar

(56) References cited:
- EP-A- 1 380 638
- US-A1- 2003 065 084
- US-A1- 2004 088 906
- DATABASE CA [Online] CHEMICAL ABSTRACTS SERVICE, COLUMBUS, OHIO, US; 1980, SHIMOMURA, KAORU: "Edible candles for birthday cake decoration" XP002407406 retrieved from STN Database accession no. 1980:469110 & JP 55 008129 B4 (SAKURA COLOR PRODUCTS CORP., JAPAN) 1 March 1980 (1980-03-01)

## Description

### FIELD OF THE INVENTION

The present invention relates to a novel candle body composition for colored flame candles and use thereof. More particularly, the present invention relates to a candle body composition for colored flame candles with improved production safety, combustion safety and flame stability, and use thereof.

### BRIEF DESCRIPTION OF ART

Conventional colored flame candles are formed of a primary combustion agent, a color-forming agent and other adjuvants, and burn with a colored flame such as red, yellow, blue, green, etc. With respect to the formulations of colored flame candles and processes for manufacturing them, there exist many patent publications. For example, Chinese Patent Application Publication No. CN 1073201A discloses a colored flame candle and manufacture thereof, said colored flame candle comprising an organic polybasic acid ester as the primary combustion agent, a higher fatty acid or higher fatty alcohol as the strength modifier, a higher fatty acid amide as the demoulding agent, metal oxides as the combustion wick modifier and metals or organic salts or complexes thereof as the color-forming agent. However, the colored flame candles disclosed in said prior arts are fragile and less flexible and burn with instable flames. In view of this, the present inventor disclosed in Chinese Patent Application No. 02124149.X a novel colored flame candle and manufacture thereof, said colored flame candle having a high strength and flexibility and thus being not easy to be crushed during its manufacture and marketing. However, the manufacture of all prior colored flame candles involves a conventional melt shaping step and thus is not suitable for DIY articles.

EP 1 380 638 A1 discloses a colored flame candle, comprises a candle body and a candle combustion wick, wherein said candle body a primary combustion agent, higher fatty acid amide, higher fatty acid triglyceride, color-forming agent, perfume and Pigment. The candles are prepared by melting the mixture of the above mentioned components, by casting said molten mixture into a mould containing a candle combustion wick therein, by cooling and subsequently demolding. JP 55008129 B discloses a candle made from solid sucrose fatty acid ester or glycerol fatty acid ester, a fat and an edible wick. The candle is prepared by heating the compositions at 60-80°C and subsequently shaping the mixture into candles.

### BRIEF SUMMARY OF THE INVENTION

Under the circumstance mentioned above, the inventors of the present invention conducted extensive investigation in the field of colored flame candles, aiming to develop a colored flame candle suitable for the manufacture requirements of DIY articles, and as the result, the inventors of the present invention found that by adding sucrose fatty acid esters, fatty acid glycerides and higher fatty alcohols during the manufacture of the candle body of the colored flame candle, it is possible to obtain a colored flame candle having a sharp flame without heat shaping. The present invention is completed based on the above finding.

An object of the present invention is to provide a novel candle body composition for colored flame candles. The candle body composition according to the present invention can be directly press-molded or provided in any containers in a form of bulk materials and by combining with a candle combustion wick, gives a colored flame candle; and furthermore, it is suitable for the manufacture requirements of DIY articles. Compared with conventional solid colored flame candles, the heat shaping step is dispensed with and thus the process for manufacturing the colored flame candles is simplified and the problem of environmental pollution is largely avoided.

Another object of the present invention is to provide a novel colored flame candle manufactured from the above-mentioned candle body composition, which has a good ignition property, a pure and sharp flame and a high retention of flame and thus is an environmentally friendly product.

Still another object of the present invention is to provide a process for manufacturing the above-mentioned colored flame candle, which does not need the heat shaping step as conventionally employed for the solid colored flame candles and thus simplifies the manufacture and largely avoids the problem of environmental pollution.

Therefore, the present invention in its one aspect provides a candle body composition for colored flame candles, comprising a primary combustion agent, a sucrose fatty acid ester as the surfactant, a fatty acid glyceride as the antioxidant and anti-mildew agent, a higher fatty alcohol as the combustion adjuvant, a color-forming agent and conventional adjuvants such as essences.

The present invention in its second aspect provides a colored flame candle, comprising a candle body formed from the above-mentioned candle body composition and a candle combustion wick.

The present in its third aspect provides a process for manufacturing the colored flame candle according to the present invention, comprising directly press-molding the above-mentioned candle body composition or providing it in a container in a form of bulk materials and then combining with a candle combustion wick.

### DETAILED DESCRIPTION OF THE INVENTION

The candle body composition for colored flame candles according to the present invention comprises the following components:

| | |
|---|---|
| Primary combustion agent | 60-95% by weight |
| Color-forming agent | 1-10% by weight |
| Sucrose fatty acid ester | 1-10% by weight |
| Fatty acid glyceride | 1-10% by weight |
| Higher fatty alcohol | 1-10% by weight |
| Powdered essence | q. s. |

wherein said percent by weight is calculated on the basis of the total weight of said composition.

The primary combustion agent which can be used in the candle body composition according to the present invention is those conventionally employed in the art and examples thereof may include paraformaldehyde, ethyl hydroxyformate, paraffins, ceresin, ethyl carbamate(urethane), sorbic anhydride, organic polybasic acid esters, polyethylene glycols, hexamethylenetetramine(urotropine), stearic acid, vinyl acetate-ethylene copolymer resins(EVA), etc., and mixtures thereof, preferably ethyl carbamate and organic polybasic acid esters such as di-C₁₋₅ alkyl oxalate, mono-C₁₋₅ alkyl succinate, tri-C₁₋₈ alkyl citrate, etc., and mixtures thereof, more preferably dimethyl oxalate, monomethyl succinate, trimethyl citrate, most preferably trimethyl citrate. The primary combustion agent is used in an amount of 60 to 95% by weight, preferably 65 to 95% by weight, more preferably 75 to 95% by weight, based on the total weight of the composition.

The sucrose fatty acid ester which can be used in the candle body composition according to the present invention is particularly sucrose C₁₀₋₃₀ fatty acid esters, more preferably mono-esters or multi-esters such as biesters, triesters and the like. In a particular embodiment of the present invention, SE series of sucrose fatty acid esters marketed by Longni Fine Chemicals Ltd., Shanghai, China are employed, in particular SE11 to SE15, more preferably SE11 (where the number such as "11" or "15" denotes a hydrophilic-lipophilic balance value(i.e. HLB value)), with the amount thereof being to 10% by weight, preferably 1 to 3% by weight, based on the total weight of the composition.

The fatty acid glyceride which can be used in the candle body composition according to the present invention is fatty acid monoglyeride, fatty acid diglyceride and fatty acid triglyceride, preferably fatty acid monoglyceride, with the amount thereof being 1 to 10% by weight, preferably 1 to 3% by weight, based on the total weight of the composition.

The higher fatty acid alcohol which be used in the candle body composition according to the present invention is C₁₀₋₃₀ fatty alcohols, preferably C₁₂, C₁₆, C₁₈ fatty alcohols or the mixture thereof, more preferably octadecanol, with the amount thereof being 1 to 10% by weight, preferably 1 to 4.5% by weight, based on the total weight of the composition.

The color-forming agent which can be used in the candle body composition according to the present invention is those conventionally employed in the art, and examples thereof may be organic salts such as formates, acetates, stearates and etc., inorganic salts such as halides(for example, chlorides, bromides, etc.), oxycholorides, nitrates, sulfates and etc., of lithium(Li), sodium(Na), potassium(K), boron(B), barium(Ba), calcium(Ca), cesium(Cs), copper(Cu), magnesium(Mg) or antimony(Sb), or complexes of the above-mentioned metals, or mixtures thereof, with the amount thereof being 1 to 10% by weight, preferably 1.5 to 8% by weight, based on the total weight of the composition.

The essences which can be used in the candle body composition according to the present invention is powdered ones conventionally employed in the art. Examples of powdered essences include powdered lemon essence, powdered vanilla essence, powdered orange essence, powdered strawberry essence and the like, with the amount thereof being that conventionally employed in the art, such as 0.001 to 0.1% by weight, preferably 0.005 to 0.05% by weight, based on the total weight of the composition.

Besides the above components, the candle body composition according to the present invention can also comprise oxidation accelerators conventionally employed in the art, such as vanadium pentoxide, chromium trioxide and etc. in amounts conventionally employed in the art.

The candle combustion wick of the colored flame candle according to the present invention can be those conventionally employed in the art, such as cotton combustion wick. The candle combustion wick to be used in the colored flame candle according to the present invention may be subjected to a pretreatment by immersing with a solution of the above-mentioned color-forming agent or other reagents according to a conventional manner in the art. In a particularly preferred embodiment, the candle combustion wick of the colored flame candle according to the present invention is pretreated by immersing with a 10% by weight aqueous hydrogen peroxide solution for 10 minutes and then air-drying, whereby the ignition property and the flame stability are substantially enhanced.

The candle body composition according to the present invention can be directly press-molded or be provided in any containers in a form of bulk materials and then combined with a candle combustion wick to form a colored flame candle. Alternatively, the candle body composition according to the present invention is suitable for the manufacture of DIY articles.

In comparison with the prior methods for manufacturing colored flame candles, the present process does not need the heat shaping step and thus is simplified and largely avoids the problem of environmental pollution.

In comparison with the prior colored flame candles, the colored flame candle according to the present invention has a good ignition property, a pure and sharp flame and a high retention of flame, and is an environmentally friendly product.

### EXAMPLES

The present invention is further demonstrated by the following examples, which shall not be construed as limiting the scope of the present invention.

### Example 1

The formulation for the candle body of a candle with a red flame is as follows:

| | |
|---|---|
| Trimethyl citrate | 94.98% |
| Lithium Propanoate | 1.5% |
| Sucrose fatty acid ester(SE11) | 1% |
| Stearic acid monoglyceride | 1% |
| Octadecanol | 1.5% |
| Powdered vanilla essence | 0.02% |

The above components are added into a container at ambient temperature and then is homogeneously mixed to form a candle body composition. The candle body composition is then added in a form of bulk materials into a mold containing a cotton combustion wick which has been previously pretreated by immersing with a 10% by weight aqueous hydrogen peroxide solution for 10 minutes and then air-drying, or directly press-molded in a mold containing such a pretreated cotton combustion wick to obtain a finished colored flame candle.

### Example 2

The formulation for the candle body of a candle with a yellow flame is as follows:

| | |
|---|---|
| Trimethyl citrate | 94.98% |
| Sodium acetate | 1,5% |
| Sucrose fatty acid ester(SE11) | 1% |
| Stearic acid monoglyceride | 1% |
| Octadecanol | 1.5% |
| Powdered lemon essence | 0.02% |

The colored flame candle is manufactured in a manner same as Example 1.

### Example 3

The formulation for the candle body of a candle with a blue flame is as follows:

| | |
|---|---|
| Trimethyl citrate | 94.98% |
| Potassium aluminum sulfate | 1.5% |
| Sucrose fatty acid ester(SE11) | 1% |
| Stearic acid monoglyceride | 1% |
| Octadecanol | 1.5% |
| Powdered orange essence | 0.02% |

The colored flame candle is manufactured in a manner same as Example 1.

### Example 4

The formulation for the candle body of a candle with a green flame is as follows:

| | |
|---|---|
| Trimethyl citrate | 94.98% |
| Boric acid | 1.5% |
| Sucrose fatty acid ester(SE11) | 1% |
| Stearic acid monoglyceride | 1% |
| Octadecanol | 1.5% |
| Powdered orange essence | 0.02% |

The colored flame candle is manufactured in a manner same as Example 1.

### Example 5

The formulation for the candle body of a candle with a violet flame is as follows:

| | |
|---|---|
| Trimethyl citrate | 94.98% |
| Potassium chloride | 1.5% |
| Sucrose fatty acid ester(SE11) | 1% |
| Stearic acid monoglyceride | 1% |
| Octadecanol | 1.5% |
| Powdered strawberry essence | 0.02% |

The colored flame candle is manufactured in a manner same as Example 1.

### Example 6

The formulation for the candle body of a candle with a magenta flame is as follows:

| | |
|---|---|
| Trimethyl citrate | 94.98% |
| Strontium nitrate | 1.5% |
| Sucrose fatty acid ester(SE11) | 1% |
| Stearic acid monoglyceride | 1% |
| Octadecanol | 1.5% |
| Powdered vanilla essence | 0.02% |

The colored flame candle is manufactured in a manner same as Example 1.

## Claims

1. A candle body composition for colored flame candles, comprising the following components:
| | |
|---|---|
| Primary combustion agent | 60-95% by weight |
| Color-forming agent | 1-10% by weight |
| Sucrose fatty acid ester | 1-10% by weight |
| Fatty acid glyceride | 1-10% by weight |
| Higher fatty alcohol | 1-10% by weight |
| Powdered essence | q. s. |
wherein said percent by weight is calculated on the basis of the total weight of said composition.

2. The candle body composition as claimed in claim 1, wherein said primary combustion agent is selected from the group consisting of paraformaldehyde, ethyl hydroxyformate, paraffins, ceresin, ethyl carbamate(urethane), sorbic anhydride, organic polybasic acid esters, polyethylene glycols, hexamethylenetetramine (urotropine), stearic acid, vinyl acetate-ethylene copolymer resins(EVA) and mixtures thereof, and is used in an amount of 65 to 95% by weight, preferably 75 to 95% by weight, based on the total weight of said composition.

3. The candle body composition as claimed in claim 2, wherein said primary combustion agent is selected from the group consisting of ethyl carbamate, di-C₁₋₅ alkyl oxalate, mono-C₁₋₅ alkyl succinate, tri-C₁₋₈ alkyl citrate and mixtures thereof.

4. The candle body composition as claimed in claim 3, wherein said primary combustion agent is trimethyl citrate.

5. The candle body composition as claimed in any one of claims 1 to 4, wherein said sucrose fatty acid ester is a mono-ester or a multi-ester, and is used in an amount of 1 to 3% by weight, based on the total weight of said composition.

6. The candle body composition as claimed in claim 5, wherein said sucrose fatty acid ester is SE11 to SE15, preferably SE11.

7. The candle body composition as claimed in any one of claims 1 to 4, wherein said fatty acid glyceride is fatty acid monoglyceride, fatty acid diglyceride or fatty acid triglyceride, and is used in an amount of 1 to 3% by weight, based on the total weight of said composition.

8. The candle body composition as claimed in claim 7, wherein said fatty acid glyceride is fatty acid monoglyceride, preferably stearic acid monoglyceride.

9. The candle body composition as claimed in any one of claims 1 to 4, wherein said higher fatty alcohol is octadecanol and is used in an amount of 1 to 4.5% by weight, based on the total weight of said composition.

10. The candle body composition as claimed in any one of claims 1 to 4, wherein said color-forming agent is organic salts or inorganic salts of lithium(Li), sodium(Na), potassium(K), boron(B), barium(Ba), calcium(Ca), cesium(Cs), copper(Cu), magnesium(Mg) or antimony(Sb), complexes of the above-mentioned metals, or mixtures thereof, and is used in an amount of 1.5 to 8% by weight, based on the total weight of said composition.

11. A process for manufacturing a colored flame candle, comprising directly press-molding the candle body composition as claimed in any one of claims 1 to 10 or providing it in a container in a form of bulk materials and then combining with a candle combustion wick.

12. A colored flame candle, obtainable by a process as claimed in claim 11, comprising a candle body composition as claimed in any one of claims 1 to 10, which is directly press-molded or provided in a container in a form of bulk materials, and a candle combustion wick.

13. The colored flame candle as claimed in claim 12, wherein said candle combustion wick is pretreated by immersing with a 10% by weight aqueous hydrogen peroxide solution for 10 minutes and then air-drying.

## Patentansprüche

1. Ein Kerzenkörper-Zusammensetzung für Kerzen mit farbiger Flamme, beinhaltend die folgenden Komponenten:
| | |
|---|---|
| primäres Verbrennungsmittel | 60-95 Gew.-% |
| farbbildendes Mittel | 1-10 Gew.-% |
| Sucrosefettsäureester | 1-10 Gew.-% |
| Fettsäureglycerid | 1-10 Gew.-% |
| höherer Fettalkohol | 1-10 Gew.-% |
| pulverisierte Essenz | in ausreichender Menge |
wobei die Gewichtsprozent-Angaben für das Gesamtgewicht der Zusammensetzung berechnet sind.

2. Die Kerzenkörper-Zusammensetzung wie in Anspruch 1 beansprucht, wobei das primäre Verbrennungsmittel ausgewählt ist aus der Gruppe bestehend aus Paraformaldehyd, Ethylhydroxyformat, Paraffinen, Zeresin, Ethylcarbamat (Urethan), Sorbinsäureanhydrid, organischen polybasischen Säureestern, Polyethylenglykolen, Hexamethylentetraamin (Urotropin), Stearinsäure, Vinylacetat-Ethylen-Copolymerharzen (EVA) und Mischungen daraus und in einer Menge von 65 bis 95 Gew.-%, vorzugsweise 75 bis 95 Gew.-%, bezogen auf das Gesamtgewicht der Zusammensetzung, eingesetzt wird.

3. Die Kerzenkörper-Zusammensetzung wie in Anspruch 2 beansprucht, wobei das primäre Verbrennungsmittel ausgewählt ist aus der Gruppe bestehend aus Ethylcarbamat, di-C₁₋₅-Alkyloxolat, mono- C₁₋₅-Alkylsuccinat, tri-C₁₋₈-Alkylcitrat und Mischungen daraus.

4. Die Kerzenkörper-Zusammensetzung wie in Anspruch 3 beansprucht, wobei das primäre Verbrennungsmittel Trimethylcitrat ist.

5. Die Kerzenkörper-Zusammensetzung wie in einem der Ansprüche 1 bis 4 beansprucht, wobei der Sucrosefettsäureester ein Monoester oder ein Multiester ist und in einer Menge von 1 bis 3 Gew.-%, bezogen auf das Gesamtgewicht der Zusammensetzung, eingesetzt wird.

6. Die Kerzenkörper-Zusammensetzung wie in Anspruch 5 beansprucht, wobei der Sucrosefettsäureester SE11 bis SE15, vorzugsweise SE11, ist.

7. Die Kerzenkörper-Zusammensetzung wie in einem der Ansprüche 1 bis 4 beansprucht, wobei das Fettsäureglycerid ein Fettsäuremonoglycerid, ein Fettsäurediglycerid oder ein Fettsäuretriglycerid ist und in einer Menge von 1 bis 3 Gew.-%, bezogen auf das Gesamtgewicht der Zusammensetzung, eingesetzt wird.

8. Die Kerzenkörper-Zusammensetzung wie in Anspruch 7 beansprucht, wobei das Fettsäureglycerid ein Fettsäuremonoglycerid, vorzugsweise Stearinsäuremonoglycerid, ist.

9. Die Kerzenkörper-Zusammensetzung wie in einem der Ansprüche 1 bis 4 beansprucht, wobei der höhere Fettalkohol Octadecanol ist und in einer Menge von 1 bis 4,5 Gew.-%, bezogen auf das Gesamtgewicht der Zusammensetzung, eingesetzt wird.

10. Die Kerzenkörper-Zusammensetzung wie in einem der Ansprüche 1 bis 4 beansprucht, wobei das farbbildende Mittel ein organisches Salz oder ein anorganisches Salz des Lithiums (Li), des Natriums (Na), des Kaliums (K), des Bors (B), des Bariums (Ba), des Kalziums (Ca), des Caesiums (Cs), des Kupfers (Cu), des Magnesiums (Mg) oder des Antimons (Sb), ein Komplex der vorstehend genannten Metalle oder Mischungen daraus ist und in einer Menge von 1,5 bis 8 Gew.-%, bezogen auf das Gesamtgewicht der Zusammensetzung, eingesetzt wird.

11. Ein Verfahren zur Herstellung einer Kerze mit farbiger Flamme, beinhaltend das direkte Druck-Formen einer Kerzenkörper-Zusammensetzung, wie in einem der Ansprüche 1 bis 10 beansprucht, oder das Bereitstellen dieser Kerzenkörper-Zusammensetzung in einem Behälter in Form von Bulkmaterialien und das anschließende Kombinieren mit einem Kerzenverbrennungsdocht.

12. Ein Kerze mit farbiger Flamme, erhältlich durch ein Verfahren wie in Anspruch 11 beansprucht, beinhaltend eine Kerzenkörper-Zusammensetzung wie in einem der Ansprüche 1 bis 10 beansprucht, welche direkt druckgeformt oder in einem Behälter in Form von Bulkmaterialien bereitgestellt ist, und einen Kerzenverbrennunsdocht.

13. Die Kerze mit farbiger Flamme wie in Anspruch 12 beansprucht, wobei der Kerzenverbrennungsdocht durch das Eintauchen in eine 10 gew.-%ige wässrige Wasserstoffperoxid-Lösung für 10 Minuten und anschließendes Lufttrocknen vorbehandelt ist.

## Revendications

1. Composition de corps de bougie pour bougies à flamme colorées, comprenant les composants suivants:
| | |
|---|---|
| agent de combustion primaire | 60 à 95 % en poids |
| agent de formation de couleur | 1 à 10 % en poids |
| ester d'acide gras de saccharose | 1 à 10 % en poids |
| glycéride d'acide gras | 1 à 10 % en poids |
| alcool gras supérieur | 1 à 10 % en poids |
| essence en poudre | q.s. |
dans laquelle ledit pourcentage en poids est calculé sur la base du poids total de ladite composition.

2. Composition de corps de bougie selon la revendication 1, dans laquelle ledit agent de combustion primaire est choisi dans le groupe constitué du parafor-maldéhyde, de l'hydroxyformiate d'éthyle, des paraffines, de la cérésine, du carbamate(uréthane) d'éthyle, de l'anhydride sorbique, des esters d'acide polybasique organiques, des poly(éthylène glycols), de l'hexaméthylènetétramine (urotropine), de l'acide stéarique, des résines copolymère éthylène-acétate de vinyle (EVA) et un de leurs mélanges, et est utilisée en une quantité de 65 à 95 % en poids, de préférence de 75 à 95 % en poids, sur la base du poids total de ladite composition.

3. Composition de corps de bougie selon la revendication 2, dans laquelle ledit agent de combustion primaire est choisi parmi le groupe constitué de carbamate d'éthyle, d'oxalate de dialkyle en C1 à 5, de succinate de monoalkyle en C1 à 5, de citrate de trialkyle en C1 à 8 et de leurs mélanges.

4. Composition de corps de bougie selon la revendication 3, dans laquelle ledit agent de combustion primaire est le citrate de triméthyle.

5. Composition de corps de bougie selon l'une quelconque des revendications 1 à 4, dans laquelle ledit ester d'acide gras de saccharose est un monoester ou un multi-ester et est utilisé en une quantité de 1 à 3 % en poids, sur la base du poids total de ladite composition.

6. Composition de corps de bougie selon la revendication 5, dans laquelle ledit ester d'acide gras de saccharose est SE11 à SE15, de préférence SE11.

7. Composition de corps de bougie selon l'une quelconque des revendications 1 à 4, dans laquelle ledit glycéride d'acide gras est le monoglycéride d'acide gras, le diglycéride d'acide gras ou le triglycéride d'acide gras et est utilisé en une quantité de 1 à 3 % en poids, sur la base du poids total de ladite composition.

8. Composition de corps de bougie selon la revendication 7, dans laquelle ledit glycéride d'acide gras est le monoglycéride d'acide gras, de préférence le monoglycéride d'acide stéarique.

9. Composition de corps de bougie selon l'une quelconque des revendications 1 à 4, dans laquelle ledit alcool gras supérieur est l'octadécanol et est utilisé en une quantité de 1 à 4,5 % en poids, sur la base du poids total de ladite composition.

10. Composition de corps de bougie selon l'une quelconque des revendications 1 à 4, dans laquelle ledit agent de formation de couleur correspond aux sels organiques ou aux sels inorganiques de lithium (Li), de sodium (Na), de potassium (K), de bore (B), de baryum (Ba), de calcium (Ca), de césium (Cs), de cuivre (Cu), de magnésium (Mg) ou d'antimoine (Sb), aux complexes des métaux mentionnés ci-dessus ou à leurs mélanges et est utilisé en une quantité de 1,5 à 8 % en poids, sur la base du poids total de ladite composition.

11. Procédé de fabrication d'une bougie à flamme colorée, comprenant le moulage sous pression directe de la composition de corps de bougie selon l'une quelconque des revendications 1 à 10 ou le fait de la fournir dans un conteneur sous une forme de matériaux en vrac, puis la combinaison avec une mèche de combustion de bougie.

12. Bougie à flamme colorée pouvant être obtenue par un procédé selon la revendication 11, comprenant une composition de corps de bougie selon l'une quelconque des revendications 1 à 10, qui est directement moulée sous pression ou fournie dans un conteneur sous une forme de matériaux en vrac et une mèche de combustion de bougie.

13. Bougie à flamme colorée selon la revendication 12, dans laquelle ladite mèche de combustion de bougie est prétraitée par immersion avec une solution de peroxyde d'hydrogène aqueuse à 10 % en poids pendant 10 minutes, puis séchage à l'air.
